

## UNITED STATES PATENT OFFICE.

CLAUDE A. O. ROSELL, OF NEW YORK, N. Y.

## CHROME TANNING-BATH.

## SPECIFICATION forming part of Letters Patent No. 759,881, dated May 10, 1904.

Original application filed August 11, 1896, Serial No. 602,431. Divided and this application filed August 26, 1902. Serial No. 121,083. (No specimens.)

To all whom it may concern:

Be it known that I, CLAUDE A. O. ROSELL, a citizen of the United States, residing at New York, in the county of New York and State 5 of New York, have invented certain new and useful Improvements in Chrome Tanning-Baths; and I do hereby declare the following to be a full, clear, and exact description of the invention, such as will enable others skilled 10 in the art to which it appertains to make and use the same.

This invention consists, essentially, in causing a skin to take up chromic oxid directly from solutions of certain salts of chromic 15 oxid, as will now be fully explained in the subjoined description and the appended claims.

The solutions of chromic-oxid salts of which I make use are thiosulfate, commonly called "hyposulfite," "sulfite," and other reducing 20 sulfur salt of chromium. These salts can be made in a number of ways, such as adding the desired acid to chromic hydrate or by decomposing chromium sulfate with a suitable salt to effect metathesis or so-called "double 25 decomposition." If a salt of calcium and barium be used, the sulfate formed is insoluble and is precipitated. If, again, a sodium salt be used, the sodium sulfate will remain in solution with the chromium salt formed. As 30 the presence of sodium sulfate in the chromium solution is entirely unobjectionable, it will be found preferable in practice to prepare the desired tanning solution by adding a suitable sodium salt to common chrome alum, 35 which is chromium potassium sulfate. A solution of chromium sulfite may be formed according to the following equation:



The reaction seems to be complete, because 40 the solution prepared as above is in no wise inferior to a solution of pure chromium sulfite. On the other hand, if a solution be made 45 of chromium sulfite and chromium sulfate it is observed that with the increase of the percentage of chromium sulfite the tanning action of the bath is improved, while the contrary effect is produced by increasing the percent-

age of chromium sulfate. This indicates 50 that no chrome-alum is left undecomposed.

Although a great many tanning solutions prepared as above will be found to give good results, such solutions differ quite considerably between themselves. It may be stated 55 that a thiosulfate solution has been found superior to a sulfite solution and a mixture of the thiosulfate and sulfite solution has been found superior to any other thus far tried.

In making use of any of the above solutions the skin may be introduced directly from the bath after washing or it may be prepared in any desired way. Thus if a skin is only partly tanned by vegetable or mineral tanning material the tanning may be completed 65 in any of the above baths of chromic-oxid salts.

If a skin is first subjected to the action of chromic acid and is afterward immersed in the above bath of chromic-oxid salt or salts, 70 two reactions will be found to take place. In the first place chromium trioxid is reduced to chromic oxid, and the reducing acid of the chromic-oxid salt is oxidized. The following equation explains the reaction:



In the second place the skin will take up chromic oxid from the solution of chromic-oxid salt.

Although the solutions of chromic-oxid salts described are initially normal, they become acid in the proportion as chromic oxid is abstracted by the skin from the chromic-oxid salt used, leaving the solvent acid behind 85 in a free state. As the acids I make use of are quite innocuous, the skins as they are tanned are not in the least injuriously affected by said liberated acids.

As before stated, the tanning-bath of chromic-oxid salt described may be used as a single bath or may also be used in connection with a chromic-acid bath.

As a single bath, the above tanning solution has the advantage of producing a more evenly 95 and thoroughly tanned and a less corroded skin than any other tanning liquid known. If this chromic-oxid liquid is used in connec-

tion with a chromic-acid bath, this process has several important advantages.

Heretofore skins have been tanned by immersion first in a bath of chromium trioxid (generally called "chromic acid") and subsequently in a reducing-bath, whereby the chromium trioxid absorbed by the skin is reduced to chromic oxid. In such processes it is necessary that the chromium-trioxid solution be made sufficiently strong to impart to the skin in one operation all the chromium which is to be combined with it, because after the chromic acid has been reduced and combined with the skin as chromic oxid the skin will not absorb additional chromic acid. Hence it is not possible to remedy skins deficiently tanned by repeating the operation. Furthermore, in such processes a portion of the chromium trioxid taken up by the skin in the first bath is washed out and lost in the second bath, and to provide for this loss an excess of chromium trioxid must be employed. For these reasons it is necessary to subject the skin in the first bath to a very strong solution of chromic acid, and since the latter is very corrosive this feature of the process is objectionable.

In my process when carried on by means of two baths it is necessary to impart to the skin in the chromium-trioxid bath only one-half to one-quarter of the chromium it is finally going to retain as combined chromic oxid, the balance of the chromium being supplied by the second or the reducing bath, consisting of a solution of the described salts of chromic oxid. It therefore follows that a skin tanned by my two-bath process is subjected to less than half the corrosive action to which a skin is subjected that is tanned by any other two-bath process—*i. e.*, being first subjected to the action of chromium trioxid and afterward to a reducing agent converting the chromium trioxid into chromic oxid.

If in any of the old two-bath chrome processes on reducing the absorbed chromium trioxid of a skin it is found to be insufficiently tanned, the skin is hopelessly ruined. By the use of my solution of a chromic-oxid salt such imperfectly-tanned skins may be saved, as they will take up sufficient chromic oxid from such a solution to effect a completion of the tanning, provided they have not been dried, in which case the hide will be tanned by substantially the following process: The skin having taken up in a chromic-acid bath less than the requisite amount of chromium to complete the tanning will be immersed in any of the old known reducing-baths, such a bath giving off sulfurous acid, hydrogen sulfid, &c. After this, before drying, it will be put into a bath containing any of the described reducing salts of chromium in quantity sufficient to complete the tanning.

Having given a general outline of the manner of forming the tanning solution, of its action and advantages, I will now give some

practical data for using the process on a large scale.

In using the chromic-oxid solution as asingle bath I proceed as follow: One hundred pounds of bated and washed skins in a wet state are immersed in fifty gallons of solution containing from two per cent. to five per cent. of chrome-alum, equal parts of sodium thiosulfate and sulfite in quantity sufficient to decompose all the chrome-alum—*i. e.*, from 0.6 per cent. to 1.5 per cent. of each—the thiosulfate, and sulfite. The skins are kept in motion in this solution and will be completely tanned in from two to four days, depending upon the character and size of the skins. The skins are then washed and finished in ordinary and approved ways. In place of adding all the chemicals at once they may be added from time to time, and in place of using a solution of the strength stated two or three baths may be used of one-half or one-third the strength, respectively.

In using the solution of chromic-oxid salt in connection with a chromium-trioxid solution I proceed as follows: One hundred pounds of bated and washed skins in a wet state are immersed in fifty gallons of a solution of three-fourths per cent. potassium bichromate and enough sulfuric acid to produce a mixture of chromic acid and potassium sulfate. After being agitated in this solution from three to twenty-four hours the skins are removed and preferably struck out, after which they are immersed in fifty gallons of liquor containing from two and one-half to four per cent. of chrome-alum and equal parts of sodium thiosulfate and sulfite in quantity sufficient to just decompose all of the chrome-alum or to leave an excess of ten per cent. to fifteen per cent. of the sodium thiosulfate and sulfite. Thus if the amount of chrome-alum be two and one-half per cent. to a solution of fifty gallons there would be added chrome-alum, ten pounds; sodium thiosulfate, three to three and one-half pounds, and sodium sulfite, three to three and one-half pounds. The skins are agitated in this solution from one to three days, depending upon the character and size of the skins, which are then washed and finished as before stated.

It should be observed that the proportions throughout the description are simply by way of example and not intended to make any limitation.

Whenever "chromium trioxid" is mentioned, it should be understood that by this term is included not only chromium trioxid in a free state, but also combinations thereof, such as the bichromates.

When any of the solutions above described is used as a single bath, it is evident that the reducing power thereof is not called into requisition. In such a case the bath, nevertheless, has the important advantage that the skins tanned are not in any way injuriously

affected by the acid set free by the operation of tanning, the only function of the acid before being set free having been to keep the chromium in solution.

5 What I claim is—

1. A tanning-bath containing an inorganic reducing sulfur salt of chromium.
2. A tanning-bath consisting essentially of a solution of chromium thiosulfate and chromium sulfite

3. A tanning-bath compounded essentially of a solution of chrome-alum, a thiosulfate and a sulfite.

In testimony whereof I have affixed my signature in presence of two witnesses.

CLAUDE A. O. ROSELL.

Witnesses:

REEVE LEWIS,  
W.M. B. ORKANE.